

1

2,870,004

## METHOD OF PRODUCING NODULAR CAST IRON

James W. Estes, New Brunswick, and Grant E. Spangler, Plainfield, N. J., assignors to Air Reduction Company, Incorporated, New York, N. Y., a corporation of New York

No Drawing. Application February 7, 1955  
Serial No. 486,714

5 Claims. (Cl. 75—51)

This invention relates to the desulfurization, upgrading and nodulizing of cast iron and particularly concerns means therefor which include provision for the addition of elemental magnesium metal to molten cast iron.

It has previously been found that an upgraded or nodular gray cast iron having properties superior to conventional gray cast iron can be produced by treating the molten iron so that, when cast, the graphite will be compacted rather than in flake form. One such treatment involves the introduction of magnesium into a molten iron bath of such composition that it would, if cast normally in the absence of any treatment, produce conventional gray cast iron in the "as cast" condition. Before such magnesium treatment will be effective to produce partial compacting (upgrading) or complete compacting (nodulizing so that substantially only spheroidal graphite exists in the cast iron), it is usually necessary to eliminate sulfur in some manner. It is highly desirable that the entire process be done so that there is a small time loss, a small heat loss, and a small cost for treating agents.

Magnesium is a well-known nodulizing-impelling or compacting agent. However, the problems involved in adding the metal itself to molten cast iron have resulted in statements in issued patents that it is impossible to add magnesium metal per se to molten cast iron without a very violent reaction and complete loss of the magnesium. The problems encountered in adding metallic magnesium to molten cast iron are due principally to the rapid conversion of magnesium to gas at the temperatures involved. It compares to dropping water on boiling grease. Another factor is the reactivity of magnesium with oxygen which results in pyrotechnic display.

The primary object of the instant invention is to provide an improved, rapid, economical injection treatment process for the upgrading and nodulizing of cast iron and an improved treating agent for use in such a process.

Another object of the instant invention is to provide an improved method for introducing elemental magnesium into molten iron.

A further object is the provision of gray cast iron treating methods and treating agents whereby desulfurizing, upgrading and nodulizing can be effected economically, quickly and consistently.

The accomplishment of the foregoing objects and others, along with the features and advantages of the in-

2

vention, will be apparent from the following description.

Generally speaking, the present invention comprises forming a molten quantity of cast iron, injecting beneath the surface of the iron a relatively dense stream of an inert gas, calcium carbide, and magnesium into the iron and then promptly casting the iron. Finely-divided calcium carbide and magnesium powder are injected and cooperatively affect the iron so that compacting of the graphite results when the iron is cast. The magnesium must be of such a size that it will pass through a 20 mesh Tyler standard sieve or screen and most (90%) will be retained on a 100 mesh screen. The magnesium powder must not exceed 15% of the mixture of calcium carbide and magnesium and preferably about 1—6 pounds of magnesium per ton of iron are injected. The carbide must be of such size that it will pass a 20 mesh screen and most (90%) will be retained on a 200 mesh screen. The density of the injection stream should be from about  $\frac{1}{4}$ —2 cubic feet of gas per pound of treating agent. The gas, of course, must be maintained at a pressure sufficient to overcome the static head of the molten iron and thus prevent entrance of the metal into the passage through which the mixture is injected. The rate of feeding can vary from about 5 to about 30 pounds of mixture per ton of iron per minute depending on the size of the ladle or quantity of iron and the type of injection apparatus. The entire injection should be performed so that not more than about 10 minutes are required for the injection. The casting should be made promptly, that is, begin casting within about 10 minutes after injection.

Since desulfurization is required in most instances, it is decidedly preferred to inject finely-divided calcium carbide by means of an injection tube in order to reduce the sulfur level to at least 0.03%, more preferably appreciably less than 0.03% or about 0.01%, and then to inject the carbide-magnesium mixture immediately through the same injection tube. In most instances, it is also preferred to inoculate the treated iron with ferrosilicon (75% silicon) or a similar inoculating agent after treating.

The amount of magnesium used will vary within the above preferred range or the operable range of  $\frac{1}{2}$  to 12 pounds per ton of iron depending on several circumstances. More magnesium is used if it is not desired to desulfurize to 0.03% sulfur with a calcium carbide treatment first or if a large casting is to be made. When desulfurizing has been done, less magnesium is injected. Furthermore, the amount of magnesium will vary depending upon whether upgraded or nodular iron is desired. For trouble-free injection and safety, the proportioning of magnesium and carbide must be such that the magnesium constitutes less than 15% of the total mixture. For effective treatment, it is necessary that the magnesium constitutes at least about 5% of the mixture. It is also considered essential that the particle size of magnesium be less than about 20 mesh but greater than 200 mesh. The apparent density of the magnesium powder preferably is about 0.7 gram per milliliter. Only slight tapping of the graduated vessel to eliminate voids was effected.

The iron which is benefited by the instant invention is an iron initially having a gray cast iron composition, that is, an iron which, if cast without treatment, would produce a cast iron having a tensile strength and the flake graphite, typical of gray cast iron. The molten iron should be less than 2750° F. at the time of injection. It is to be noted that the product resulting from the instant invention will normally contain retained magnesium in an amount which by itself would be insufficient to produce the type of product obtained. The fact that less retained magnesium is necessary to produce a given structure is due to the action of the carbide. The apparatus for injecting the instant treating agent can be, for example, the screw feeder device shown in the Hulme Patent No. 2,577,764; the batch feeder as disclosed in the Cleeny-Rowen U. S. application Serial Number 430,864; or the fluidizer injection device shown in the Muller, Fisher and Hulme U. S. application Serial Number 324,998 (all assigned to the assignee of the instant application). All of these apparatus are so built as to provide a solid gas stream having a density of about  $\frac{1}{4}$  to 2 gas-to-solid ratio (cubic feet of gas per pound of mixture). The preferred inert gas which is used to inject the instant treating agents and calcium carbide is dry nitrogen. Other gases which can be used are helium, argon, and carbon dioxide. The term, inert gas, herein means a gas which does not react with magnesium or iron under the described conditions.

The instant treating agent is prepared by intimately mixing by any conventional means between 10 to 17 parts of finely-divided calcium carbide with 1 to 2 parts magnesium powder so that the magnesium constitutes less than 15%. The calcium carbide is a commercial grade calcium carbide, quite free of impurities, as made in electric arc furnaces from calcium oxide and high quality coke. As above mentioned, the calcium carbide is sized so that all of it passes through a 20 mesh screen and no more than about 25% of it passes through a 100 mesh screen (standard Tyler screen). The magnesium powder is in the form of very small irregular chip-like particles. Under the microscope, these particles have irregular edges which are frequently rolled-up. These magnesium particles must be sized, as above mentioned, so that they pass a 20 mesh screen and 90% are retained on a 100 mesh screen. A typical screen analysis of the magnesium was 100% minus 20; 86.7% minus 48; 42% minus 65; and 6.8% minus 100. The calcium carbide particles are also graduated as to size although more particles are finer than with the magnesium. The quantities of the components of the instant treating agent which are used per ton of gray cast iron range between 10 and 80 pounds for calcium carbide and between  $\frac{1}{2}$  to 12 pounds for magnesium. In any event, the magnesium must not exceed 15% of the total.

In the initial tests made with small particles of magnesium, it became apparent that preventing plugging of the injection tube was a major consideration independent of hazards as to the amount of magnesium or the efficiency of the injection. With the proportioning and particle sizes herein taught, plugging of various sized injection tubes is substantially avoided. Thus, the instant features resolve both the problem connected with the feeding of magnesium particles through a red-hot carbon injection tube to beneath the surface of molten cast iron and the hazardous problem of violence involved when a quantity of magnesium contacts molten cast iron which is above the vaporization temperature of magnesium. This latter problem primarily involves a change of state hazard, due to a solid being suddenly converted to a gas occupying many times the volume. There is the further hazard of magnesium oxidizing at the surface or flaring. The present invention minimizes this flaring problem since the magnesium is dispersed beneath the surface, is effectively dissolved into the iron

and is partially shielded at the surface by the slag formed by the carbide. It is to be appreciated also that the instant mixture contributes to safety in storage and handling. Segregation of the magnesium during feeding is also minimized due to the interlocking of the rough edges of the magnesium and carbide.

To illustrate in detail the application of the process provided by the instant invention, a preferred embodiment thereof will be described. A molten cast iron bath was established which, if then cast, would result in gray cast iron containing flake graphite. This bath was injected with 16 pounds of carbide through a carbon injection tube in order to reduce the original sulfur percentage of 0.082 and further benefit the iron. Next an intimate and homogeneous mixture of magnesium and calcium carbide was injected immediately through the same tube. Dual hoppers can be used or fast recharging can be done so that not more than one minute is required between injections. The mixture was proportioned 36 pounds of carbide per ton of iron to 4 pounds of magnesium per ton of iron so that the magnesium constituted about 10%. Dry nitrogen was used as the carrier gas. The injection was at the rate of 28.5 pounds of mixture per ton of iron per minute. The gas to solid ratio was 0.418 cubic feet per pound. The carbon injection tube was immersed more than  $\frac{1}{2}$  the depth of the basic-lined vessel. A depth of at least 6 inches is essential. The temperature of the iron was about 2700° F. Ferrosilicon (75% silicon) was added immediately after injection in an amount equivalent to one percent per ton. The iron was cast within 3 minutes after completion of the injection. A fully nodular cast iron was obtained. This iron had an ultimate tensile strength of 62,250 p. s. i., a Brinnell hardness number of 143, an elongation of 18.5% in two inches, and a chill of  $2\frac{1}{2}$  of an inch. The foregoing test is test number 882-1 in the following tables which give comparable data for other tests as well as chemical analyses.

Some cast irons contain small amounts of elements which are sometimes referred to as subversives or interfering elements. The elements lead, arsenic, tin, and antimony are some of the elements believed to be subversive. When such irons are encountered as can be determined by results which are inconsistent with those shown as generally obtained with treating with calcium carbide and magnesium, it is preferred to incorporate a small amount of rare earths oxides (REO) in the carbide-magnesium mixture. Apart from the foregoing consideration, it is preferred to use REO when the compacted graphite as herein described is desired and small quantities of magnesium are used since rare earths effect compacting. Between one and two pounds of REO per ton of iron are preferred. The REO is finely-divided, being at least 20 by 0 mesh size. The REO contains about 50% cerium oxide, 20% lanthanum oxide, and the remainder is decreasing percentages of the other rare earth substances. This composition is typical of the rare earths as found in nature. The term rare earth substance is intended to mean materials such as the described REO or rare earth derivatives in their naturally occurring proportions.

In the preferred embodiment wherein desulfurizing and benefiting, such as deoxidation, is first effected by the injection of calcium carbide and then the remaining and principal compacting treatment is immediately done using magnesium and calcium carbide or magnesium, calcium carbide, and REO, the preferred quantity of carbide which is added is somewhat in excess of 10 pounds of carbide per pound of sulfur to be removed so that the sulfur level of less than 0.03% is rapidly obtained and the carbide can affect the iron in a beneficial way and make it more receptive to the effect of magnesium. The following table shows the proportioning, other conditions, and results when carbide treatment is effected first.

Table I

| Test No.   | Injection Mix (Lbs./Ton) |       |      | Temp., °F. | Chemical Analysis |       |      |     |        |         |      | Properties |          |          |        |         |
|------------|--------------------------|-------|------|------------|-------------------|-------|------|-----|--------|---------|------|------------|----------|----------|--------|---------|
|            | CaC <sub>2</sub>         | REO   | Mg   |            | Percent Late FeSi | T. C. | Si   | Mn  | Base S | Final S | P    | C. E.      | U. T. S. | B. H. N. | Elong. | Chill % |
| 815-1----- | { 20<br>45               | ----- | 5.0  | 2,680      | 0.75              | 3.58  | 2.68 | .22 | .013   | .006    | .03  | 4.47       | 69,200   | 163      | 18.5 x | 20      |
| 867-1----- | { 20<br>17               | 1.0   | 2.0  | 2,650      | 0.75              | 3.59  | 2.26 | .08 | .088   | .003    | .043 | 4.34       | 69,800   | 163      | 7.8 x  | 32      |
| 879-1----- | { 16<br>34               | 2.0   | 4.0  | 2,700      | 1.00              | 3.56  | 2.57 | .12 | .082   | .003    | .028 | 4.43       | 63,200   | 149      | 18.0 x | 48      |
| 880-1----- | { 16<br>34               | 2.0   | 4.0  | 2,700      | 1.00              | 3.60  | 2.54 | .12 | .107   | -----   | .022 | 4.45       | 64,200   | 146      | 17.0 x | 36      |
| 881-1----- | { 16<br>20.2             | 1.19  | 2.38 | 2,700      | 1.00              | 3.56  | 2.57 | .14 | .100   | -----   | .027 | 4.43       | 64,000   | 155      | 19.0 x | 32      |
| 882-1----- | { 16<br>36               | ----- | 4.0  | 2,700      | 1.00              | 3.66  | 2.43 | .14 | .082   | -----   | .028 | 4.48       | 62,250   | 143      | 18.5 x | 20      |
| 883-1----- | { 16<br>22.6             | 1.33  | 2.66 | 2,700      | 1.00              | 3.55  | 2.32 | .30 | .113   | -----   | .033 | 4.33       | 81,300   | 186      | 11.5 x | 24      |
| 884-1----- | { 16<br>34               | 2.0   | 4.0  | 2,700      | 1.00              | 3.55  | 2.46 | .33 | .103   | -----   | .036 | 4.38       | 67,750   | 162      | 9.5    | 32      |
| 903-1----- | { 16<br>26               | 1.0   | 3.0  | 2,700      | 1.00              | 3.57  | 2.44 | .37 | .096   | -----   | .034 | 4.38       | 66,850   | 159      | 17.5 x | 10      |

The data under the heading "Chemical Analysis" refers to the final percent analysis as to silicon, manganese and phosphorus. Base (initial) and final sulfur percent are both shown. The other data include pounds of the materials injected per ton of iron and properties such as ultimate tensile strength (U. T. S.) and elongations (Elong.) as percentage in two inches. The top quantity of carbide in each line is that used for initial desulfurizing and benefiting. The second, or bottom, quantity is the amount of carbide incorporated into the compacting mixture. The abbreviations T. C. and C. E. respectively refer to total carbon and carbon equivalent. The temperature is that of the iron at the beginning of the treatment. The term, percent late FeSi, refers to the addition of ferrosilicon (75% silicon) as a percentage of the iron being treated. The ferrosilicon was added by relarding, although it can be injected. When no value is given, ferrosilicon was not added.

Flakes were eliminated in substantially all of the tests herein described. It was quite apparent that the wormy graphite was a strength-contributing factor. Examples 25 of irons having compacted graphite as a mixture of nodules and wormy formations are tests No. 884-1 about 60% nodules (supra); No. 871-1 about 50% nodules (infra); and No. 872-1 about 50% nodules (infra). In 30 general, the higher the percentage of nodules, the higher the tensile strength.

Sometimes it may be desirable to treat with mixtures of 35 magnesium and calcium carbide without immediate prior carbide treatment. This can be done either when low sulfur iron is available or when, with higher sulfur iron, there are advantages in using only one mixture comprised of magnesium and carbide. The following Table II shows the proportioning, conditions, and results when 40 magnesium and carbide were injected together.

Table II

| Test No.   | Injection Mix (Lbs./Ton) |     |                   | Temp., °F. | Chemical Analysis |      |     |        |         |      |       | Properties |          |        |         |
|------------|--------------------------|-----|-------------------|------------|-------------------|------|-----|--------|---------|------|-------|------------|----------|--------|---------|
|            | CaC <sub>2</sub>         | Mg  | Percent Late FeSi |            | T. C.             | Si   | Mn  | Base S | Final S | P    | C. E. | U. T. S.   | B. H. N. | Elong. | Chill % |
| 783-3----- | 25                       | 3.3 | 2,740             | 0.60       | 3.61              | 2.34 | .42 | .077   | .015    | .11  | 4.42  | 51,300     | 167      | 2.0 x  | 12      |
| 781-1----- | 36                       | 4.0 | 2,595             | -----      | 3.61              | 2.08 | .43 | .083   | .008    | .11  | 4.34  | 59,300     | 285      | 0 x    | 118     |
| 781-2----- | 36                       | 4.0 | 2,595             | 0.60       | 3.61              | 2.48 | .43 | .083   | .009    | .11  | 4.47  | 78,200     | 176      | 7.5 x  | 10      |
| 789-3----- | 44                       | 6.0 | 2,715             | 0.75       | 3.15              | 2.57 | .42 | .088   | .017    | .11  | 4.04  | 62,300     | 211      | 2.0    | 12      |
| 782-2----- | 34                       | 6.0 | 2,650             | 0.60       | 3.45              | 2.42 | .51 | .087   | .013    | .11  | 4.20  | 81,400     | 174      | 9.0 x  | 20      |
| 791-3----- | 44                       | 6.0 | 2,550             | 0.75       | 3.18              | 2.66 | .44 | .082   | .012    | .11  | 4.10  | 79,500     | 187      | 8.0 x  | 16      |
| 792-3----- | 44                       | 6.0 | 2,500             | -----      | 3.42              | 2.21 | .21 | .023   | .006    | .03  | 4.14  | 70,350     | 203      | 3.5 x  | 118     |
| 792-4----- | 44                       | 6.0 | 2,500             | 0.60       | 3.42              | 2.58 | .21 | .023   | .006    | .03  | 4.28  | 64,400     | 149      | 21.8 x | 14      |
| 871-1----- | 18                       | 2.0 | 2,700             | 1.40       | 3.41              | 2.77 | .03 | .006   | .006    | .024 | 4.34  | 56,250     | 143      | 8.7    | 18      |
| 878-1----- | 36                       | 4.0 | 2,700             | 1.00       | 3.40              | 2.55 | .04 | .022   | .003    | .027 | 4.26  | 63,850     | 149      | 21.0 x | 32      |
| 858-1----- | 36                       | 4.0 | 2,700             | 1.00       | 3.37              | 2.62 | .16 | .013   | .004    | .03  | 4.24  | 66,200     | 163      | 8.5    | -----   |

In test No. 883-1, the magnesium was 65 by 100 mesh. This magnesium powder passed the first screen and was retained on the second screen. This test shows the effectiveness of the carbide in cooperation with very small particles of magnesium.

The chill figure in the above and following tables was obtained by casting into a sand mold against a graphite block as a base. The wedge formed was 3½ inches high, ⅜ of an inch wide at the top and ⅛ of an inch at the bottom. The tabulated figures are the depth (height) of the chill from the bottom of the wedge contacting the block in 32nds of an inch.

The irons in the above and following tables which have an "x" after the elongation values were fully nodular, that is, the graphite was present only as nodules. The other irons were upgraded, that is, not flaky but having compacted graphite in the form of nodules and wormy-like formations (thick, short strands).

As indicated by Table II, it is apparent that it is possible to desulfurize and compact a relatively high base sulfur iron by using only a mixture of magnesium and carbide. For instance, test No. 781-2 shows such a result and gave a fully nodular iron. It is to be noted that compacted graphite is obtained with temperatures as low as 2500° F. Tests No. 781-2 and 791-3 show this result and the making of fully nodular iron. Tests No. 783-3 and 858-1 respectively gave irons having 14% and 95% of the graphite in the form of nodules, the remainder of the graphite being wormy graphite.

The following table III indicates the proportioning, other conditions, and results when using magnesium, REO and calcium carbide without immediate prior desulfurizing since the initial sulfur level was low in all tests as can be easily, and preferably is, effected by carbide treatment.

Table III

| Test No.   | Injection Mix<br>(Lbs./Ton) |     |     | Temp.,<br>° F. | Chemical Analysis       |       |      |     |           |            |      |       | Properties |          |        |            |
|------------|-----------------------------|-----|-----|----------------|-------------------------|-------|------|-----|-----------|------------|------|-------|------------|----------|--------|------------|
|            | CaC <sub>2</sub>            | REO | Mg  |                | Percent<br>Late<br>FeSi | T. C. | Si   | Mn  | Base<br>S | Final<br>S | P    | C. E. | U. T. S.   | B. H. N. | Elong. | Chill<br>% |
| 836-1----- | 20                          | 1.0 | 2.0 | 2,700          | 1.60                    | 3.36  | 3.33 | .37 | .018      | .006       | .04  | 4.49  | 56,800     | 167      | 5.0    | 4          |
| 839-1----- | 20                          | 1.0 | 1.0 | 2,700          | 1.60                    | 3.47  | 3.26 | .32 | .015      | .007       | .04  | 4.56  | 55,400     | 156      | 5.0    | -----      |
| 848-1----- | 17                          | 1.0 | 2.0 | 2,700          | 0.75                    | 3.38  | 2.23 | .18 | .018      | -----      | .025 | 4.12  | 54,350     | 140      | 5.0    | 26         |
| 850-1----- | 17                          | 1.0 | 2.0 | 2,700          | 1.00                    | 3.76  | 2.45 | .17 | .010      | -----      | .025 | 4.58  | 59,100     | 139      | 14.5   | 12         |
| 856-1----- | 34                          | 2.0 | 4.0 | 2,700          | 1.00                    | 3.30  | 2.47 | .15 | .015      | .005       | .029 | 4.12  | 65,700     | 152      | 18.5x  | 32         |
| 872-1----- | 17                          | 1.0 | 2.0 | 2,700          | 1.40                    | 3.38  | 2.76 | .17 | .017      | .006       | .031 | 4.31  | 53,800     | 150      | 5.0    | 16         |

An upgraded iron was also obtained from a low sulfur hypoeutectic iron by injecting 15 pounds of carbide per ton of iron and 1 1/4 pounds of magnesium per ton, with a 0.5% late ferrosilicon inoculation. The magnesium constituted about 7.5% of the mixture. The tensile strength was almost doubled although no nodules were made. This test indicates the preferred lower quantity and necessary proportion for magnesium, that is, about one pound per ton of cast iron and about 5% of the mixture.

It is to be noted that the instant invention is very useful for obtaining a nodular iron having a low silicon content, that is, less than 2.5% silicon, because the only silicon added is in the inoculation. Such an iron gives a higher impact strength than many nodular irons having a greater percentage of silicon and can be used to replace brass in some applications.

By reference to the tests set forth in the above tables, it can be seen that many types of cast irons can be produced, ranging from fully nodular to upgraded irons having tensile strengths of about 50,000 p. s. i. It is to be noted that these tests were made with cast irons which are at or near the eutectic point, 4.3% carbon equivalent (C. E.) which is the carbon percentage plus 1/3 of the sum of the percentages for silicon and phosphorus. The preferred C. E. range is 4.0 to 4.6 although the instant invention is useful in treating irons within the range of 3.8 to 5. It is to be understood that basic-lined or acid-lined vessels or fore-hearth type structures with either type of lining can be used.

All mesh sizes herein specified are standard Tyler screen sizes. All percentages are weight percentages.

It is to be understood that the instant invention comprehends injecting a mixture of magnesium powder, finely-divided calcium carbide and a small amount of other finely-divided substances such as rare earth substances, magnesium oxide or graphite. However, the carbide should always constitute more than 80% of the mixture and the magnesium must not exceed 15% of the total. In a test identical to No. 783-3, except for the omission of the late ferrosilicon addition, the simultaneous injection of carbide, magnesium, and graphite (about 0.3% graphite in relation to the iron) was effected with good results.

The aforementioned quantities of magnesium and other agents, the manner of introducing, and the size of the particles provide for adding magnesium without excessive violence and without excessive magnesium flare at the surface of the cast iron and yet provide an improved, rapid and economical treatment. It is to be noted that the granular-like slag similar to the usual slag from carbide alone, is believed to be helpful in minimizing magnesium flare.

It is to be appreciated that the instant invention provides an improved practical method for making upgraded and nodular irons economically. Large expensive metallic additions are avoided causing less chilling of the melt, low silicon nodular irons can be readily made, unwanted alloying elements are not present to be recirculated in foundry returns, the cost of treatment is significantly

lowered below that of alloy addition treatment, and the treated metal and foundry ladles are free of any drossy slags or scum. Lower temperatures of the iron at the time of treating do not reduce the effectiveness of the carbide-magnesium treatment. It is also to be appreciated that the instant invention substantially eliminates or minimizes the violence and flaring sometimes encountered in adding elemental, pure magnesium and, equally important, substantially avoids plugging in the immersed injection tube.

As persons skilled in the art will understand, modifications and variations of and in the present invention as above described in detail can be resorted to without departing from the scope of the invention as defined in the appended claims.

We claim:

1. A method for producing cast iron containing compacted graphite which comprises establishing a bath of molten cast iron composition which if cast without treatment would contain flake graphite; continuously introducing a stream of an inert gas and a mixture of finely divided solid calcium carbide and elemental magnesium particles into said bath beneath the surface thereof; said magnesium particles constituting about 5-15% of the weight of said mixture; said carbide and magnesium particles being of a fineness sufficient to pass a 20-mesh screen and incapable of passing a 200-mesh screen; the ratio of said gas to said solid mixture being about 1/4 to 2 cubic feet of gas per pound of mixture; and promptly casting the resulting treated metal to obtain a casting containing a substantial amount of compacted graphite, said mixture effecting a product improvement which is significantly greater than the sum of the improvement that would be obtained by treatment with the same amount of said calcium carbide alone plus the improvement that would be obtained by treatment with the same amount of said elemental magnesium alone.

2. The method according to claim 1 in which said stream contains a small amount of a finely divided rare earth substance, said amount constituting about one to two pounds per ton of said molten iron.

3. The method according to claim 1 in which a stream of inert gas and finely divided calcium carbide particles are injected into said iron immediately prior to said step of injecting said calcium carbide and said magnesium, and continuing the injection of said stream of inert gas and calcium carbide particles until the sulfur level is below 0.03%.

4. A composition for treating molten cast iron at normal founding temperature to produce a cast iron containing compacted graphite which comprises a mixture of finely divided calcium carbide particles and elemental magnesium particles; said magnesium particles constituting between 5% to 15% of said agent; said calcium carbide and magnesium particles being of a fineness sufficient to pass through a 20-mesh screen and being of a size which is substantially entirely retained on a 200-mesh screen; and said calcium carbide and elemental magnesium particles being thoroughly mixed.

5. The composition as defined in claim 4 and being

further characterized in that a small amount of finely divided oxides of rare earths is thoroughly mixed therein, said amount constituting about one to two pounds per ton of said molten iron.

References Cited in the file of this patent

UNITED STATES PATENTS

|           |              |               |    |
|-----------|--------------|---------------|----|
| 2,488,512 | Morrogh      | Nov. 15, 1949 | 5  |
| 2,527,498 | Jordan       | Oct. 24, 1950 | 10 |
| 2,529,346 | Mills et al. | Nov. 7, 1950  |    |
| 2,530,368 | Jordan       | Nov. 21, 1950 |    |

|           |           |           |           |           |
|-----------|-----------|-----------|-----------|-----------|
| 2,538,263 | 2,543,853 | 2,563,859 | 2,577,837 | 2,577,764 |
| 2,622,022 | 2,652,324 | 2,661,281 | 2,749,990 |           |
|           |           |           |           | 497,020   |
|           |           |           |           |           |

|              |       |                |
|--------------|-------|----------------|
| Offenhauer   | ----- | Jan. 16, 1951  |
| Jordan       | ----- | Mar. 6, 1951   |
| Mills et al. | ----- | Aug. 14, 1951  |
| Zifferer     | ----- | Dec. 11, 1951  |
| Hulme        | ----- | Dec. 11, 1951  |
| Crome        | ----- | Dec. 16, 1952  |
| Hignett      | ----- | Sept. 15, 1953 |
| Morrogh      | ----- | Dec. 1, 1953   |
| Morrogh      | ----- | May 29, 1956   |

FOREIGN PATENTS

|        |       |              |
|--------|-------|--------------|
| France | ----- | Nov. 3, 1950 |
|--------|-------|--------------|